

(No Model.)

J. R. HEBAUS.

## APPARATUS FOR EXTRACTING PRECIOUS METALS

No. 603,904.

Patented May 10, 1898.



**WITNESSES :**

Edward Thorpe.  
C. R. Ferguson

INVENTOR  
J. H. Heebaus  
BY manu B  
ATTORNEYS.

ATTORNEYS.

# UNITED STATES PATENT OFFICE.

JOSEPH R. HEBAUS, OF BUTTE, MONTANA, ASSIGNOR OF ONE-HALF TO  
FREDERICK P. CONROY, OF SAME PLACE.

## APPARATUS FOR EXTRACTING PRECIOUS METALS.

SPECIFICATION forming part of Letters Patent No. 603,904, dated May 10, 1898.

Application filed May 21, 1897. Serial No. 637,509. (No model.)

*To all whom it may concern:*

Be it known that I, JOSEPH R. HEBAUS, of Butte, in the county of Silver Bow and State of Montana, have invented a new and Improved Apparatus for Extracting Precious Metals, of which the following is a full, clear, and exact description.

This invention relates to an apparatus for extracting precious metals—such, for instance, as gold and silver—from ores, tailings, and other compounds; and the object is particularly the extraction of gold and silver from sulfid ores carrying gold or silver in the metallic state or as sulfids, hematite carrying a proportion of precious metals, and also in general oxid ores of the base metals—such as iron, copper, lead, and zinc—which contain an admixture of gold or silver, or both.

The invention consists in the construction and combination of the various parts and details, as will be fully described hereinafter, and defined in the appended claims.

Reference is to be had to the accompanying drawing, forming a part of this specification, in which the figure represents a vertical section of an apparatus by means of which my process may be carried out.

Referring to the drawing, 1 designates a tank of any desired construction and open at its top. This tank has a lining 2, of amalgamated copper, which constitutes the cathode. Within the tank agitators are arranged. These agitators consist of shafts 3 4, having disks or arms 5 6 at the lower end, of insulating material—such, for instance, as hard rubber or metal covered with rubber. The object in making the arms or disks of insulating material is to obviate any possibility of short-circuiting should the agitators by some accident or bridging form a connection with the bottom of the tank. Such short-circuiting would cause the destruction of both the anode and cathode and possibly the whole machine. Extended radially from the shaft are arms 7, consisting of iron or similar metal, and these arms will constitute the anode. The shaft 3 is provided at its upper end with a pinion 8, and the shaft 4 is provided at its upper end with a pinion 9. These pinions 8 and 9 engage with a gear-wheel 10, mounted

on a shaft 11, having bearings in a frame 12, mounted on the tank. Secured to the shaft 11 is a bevel-gear 13, meshing with a bevel-pinion 14 on a driving-shaft 15, to which a drive-wheel 16 is attached. The shafts 3 and 4 have bearing at their upper ends in a bar 9<sup>a</sup>, mounted to turn on the lower end of the shaft 11, so that the agitators will not only revolve on their own axes, but will travel around the tank to thoroughly stir the contents of the tank.

The cathode or amalgamated copper lining 2 is attached to a source of electricity, here shown as a battery 17, by means of which a wire 18 and the anodes consisting of the shafts 65 3 and 4 and the arms thereon are connected to said source of electricity by a wire 19. As before stated, I employ an electric current of very low tension; but I increase the surface of the anode and cathode to as large an extent as possible, and thus I am enabled to deposit the precious metals as soon as they are dissolved upon the cathode, where the metal may be recovered as an amalgam.

In the operation of my invention I charge 75 the tank with the required quantity of water and set the agitators in rotary motion. I then gradually introduce the ore, which should be pulverized, and I gradually introduce salt, caustic soda, lime, or other alkaline earths 80 until litmus-paper turns blue by testing the whole mass. The lime, salt, and caustic soda cannot be used in equal proportions. Ores which carry but little silver do not require salt. Ores which carry silver in quantity require 85 one pound of salt to the ounce of silver. In proportion to one pound of caustic soda I use sixteen pounds of lime. I dissolve salt, caustic soda, and lime in water in the proportions stated above. Only caustic soda and lime are 90 necessary for alkalinity. Now the charge is ready to receive the chemical solution, which consists of from one-fourth to three-fourths per cent. of cyanid of potassium or other cyanogen-yielding substances. At the time the 95 chemical solution is introduced the electric current must be turned on. Diluted bromine and sodium dioxid are added during the operation, care being taken to have the potassium cyanid in excess and not to add the bro- 100

- min and sodium dioxid faster than the cyanogen is set free. In this manner my process becomes a continuous one of dissolving the precious metals from the ore, immediately precipitating the same, sending the solution freed from its metals into the charge of dissolving ore, regenerating continuously the solvent for further action on the undissolved precious metals still contained in the ore.
- 5 10 After the ore shall have been treated a sufficient length of time—say from two to three hours—the ore and solution is drawn off through the valve-controlled outlet 20. This ore and solution will be drawn off into another vat, where it may settle, and after it shall have sufficiently settled the solution may be removed from the vessel and used over again with the addition, if necessary, of a new supply of cyanid of potassium.
- 15 20 The advantage in treating ores and tailings with cyanid of potassium, bromin, and sodium dioxid, in conjunction with an electric current, lies in the fact that the precious metals are attacked more energetically in conjunction with a current of electricity than without one. The gold and silver contents in tailings from an amalgamation process are mostly coated with amalgam, and no solution of cyanid of potash is able to penetrate
- 25 30 this amalgam in order to bring out the gold; but electricity in connection with the cyanid of potash will cause the dissolving and precipitation of the gold or silver, and, further, the electrical current saves cyanid of potash,

which would be destroyed by zinc precipita- 35  
tion.

In case I have to deal with free-milling ore I cover the bottom of the tank with mercury, but do not require said mercury with base compounds.

40 I am aware that cyanid of potassium, bromin, and sodium dioxid, in conjunction with an electric current, have been used for the extraction of gold and silver from ores, and such I do not claim.

45 Having thus described my invention, I claim as new and desire to secure by Letters Patent—

1. An apparatus for extracting precious metals from their ores comprising a tank having 50 an amalgamated copper lining forming a cathode and a multiplicity of agitators each rotating on its own axis and at the same time traveling around the tank, the said agitators forming an anode, and an electric circuit, substantially as specified.

2. The tank having a conducting-plate adapted to form a cathode, a rotatable frame, a conducting-agitator mounted rotatably on the frame and upon an axis eccentric to that 60 of the frame, means for connecting the agitator and plate to a source of electric current, and means for rotating the agitator and frame, substantially as specified.

JOSEPH R. HEBAUS.

Witnesses:

FREDERICK P. CONROY,

ALBERT G. CORBETT.